

Aug. 15, 1950

H. C. GERRISH ET AL  
OXIDIZER AND DESICCATOR UNIT

**2,518,460**

Original Filed Oct. 23, 1943



FIG. 2



1000



HAROLD C. GERRISH &  
J. LAWRENCE MEEM, JR.

Inventor

၁၃၁

Murray O. Hayes

Attorney

## UNITED STATES PATENT OFFICE

2,518,460

## OXIDIZER AND DESICCATOR UNIT

Harold C. Gerrish and James Lawrence Meem, Jr.,  
Cuyahoga County, OhioOriginal application October 23, 1943, Serial No.  
507,388. Divided and this application March 7,  
1945, Serial No. 581,539

1 Claim. (Cl. 23—254)

(Granted under the act of March 3, 1883, as  
amended April 30, 1928; 370 O. G. 757)

1

This invention relates in general to low temperature oxidation of exhaust gases from internal combustion engines in connection with thermal-conductivity cells used in gas analysis.

As heretofore known, one type of gas analysis apparatus used for indicating the fuel-air ratio of the mixture fed to internal combustion engines over the ignitable range of mixtures, is based upon the oxidation of the products of incomplete combustion by passing them through copper oxide heated to a high temperature, in the neighborhood of 900 to 1500 degrees Fahrenheit, and then determining the percentage of the several gas constituents in the resulting mixture, by means of the thermal conductivity cells, similar to those shown, for example, in prior Patent No. 2,298,288, issued October 13, 1942, to Gerrish and Reuter. This procedure requires the use of a furnace of some sort to attain these temperatures. In some cases, the furnace used is constituted by the exhaust stack of the engine, within which the copper oxide may attain the proper operating temperature. Such a procedure, however, makes servicing the oxidizer difficult whether the engine be in an airplane or other vehicle, in a laboratory, or elsewhere. The primary object of our invention is to provide an oxidizing substance that will completely oxidize the hydrogen in the exhaust gases to water, the carbon monoxide to carbon dioxide, and the saturated and unsaturated hydrocarbons to carbon dioxide and water while the exhaust gases are at room temperature or lower and without the use of a furnace or device for heating the oxidizing agent to some higher temperature.

A further object is to devise means whereby samples of the gases of combustion either from the exhaust stack of any cylinder of a multi-cylinder engine or from a collector ring into which all the individual cylinders discharge their exhaust gases, may be readily oxidized at a distance from the position of gas sampling without the difficulties necessarily encountered in inserting a high temperature oxidizer in these gas sampling positions.

Further and more specific objects of this invention will become apparent from the following description thereof, having reference to the accompanying drawings, wherein:

Fig. 1 is an illustrative embodiment of our invention diagrammatically showing the gas circuit from the position of sampling in the exhaust stack, through the desiccator, the low temperature oxidizer, the thermal conductivity cells of

the analyzer or bridge circuit, and through the bubbler whereby the rate of gas flow is controlled;

Fig. 2 is a longitudinal section of one form of low temperature oxidizer unit, and

5 Fig. 3 is a section taken at 3—3 of Fig. 2. It has been customary, in the type of analyzer referred to, to pass the completely oxidized gases through a hot-wire instrument, whose operation depends upon the variation of the thermal conductivity of the oxidized gases of combustion with mixture strength, thereby to determine the mixture strength of the particular fuel-air mixture used in producing the gases. The instrument is essentially a Wheatstone bridge whose 10 resistance elements consists partially or totally of filaments whose temperatures and therefore electrical resistances are influenced by the thermal conductivity of the gases surrounding them, which conductivity is dependent on the percentage of CO<sub>2</sub> in the gas, and this percentage is in turn dependent on the fuel-air mixture fed to the engine, provided all the carbon has been oxidized into CO<sub>2</sub> and all the hydrogen into water.

For the oxidation of the exhaust gases, various 15 oxidizers such as copper oxide, Hopcalite, etc., have been used, but the oxidation, to be effective, requires high temperatures.

It has been found that, by using oxidizing agents of the type to which our invention relates, the oxidation could be performed at room or lower temperatures, thus overcoming the difficulties of high temperature oxidation requirements.

The gas circuit used with these oxidizers, 20 one form of which is shown in Fig. 1, is much simpler and easier to service with the oxidizing material than that used with any of the high temperature oxidizers. The oxidizers used in this invention are not merely catalysts but oxidizing agents. The oxygen for the reaction is supplied 25 from the oxide mixtures themselves, and therefore it is not necessary to introduce some extraneous gas such as air to furnish the desired oxygen and thus vary the gas composition. We have 30 found several substances which are well adapted to use in our circuit. They are defined in a co-pending application Serial No. 507,388, filed October 23, 1943, of which the present application is a division, now abandoned.

These substances are various combinations of 35 the oxides of silver, manganese, copper, cobalt, nickel, iron, mercury and cerium. The following three specific examples illustrate some of the preferred methods of preparing these oxidizing agents and it is to be understood that the inven-

tion is not to be limited to the specific mixtures and methods described.

*Example 1.*—A product consisting of the mixed oxides of silver, manganese and copper was prepared as follows: To a portion of 37 grams of silver nitrate in 2 litres of distilled water, 75 grams of a finely powdered mixture of copper oxide and manganese dioxide known commercially as "Hopcalite" were added. Silver oxide was precipitated in the presence of the "Hopcalite" by the addition of sodium and potassium hydroxide. After settling, the material was washed by decantation six times with distilled water and filtered by suction.

The precipitate was dried for two hours at 75° C., pressed to a cake in a hydraulic press, and dried four hours longer at 75° C. After the second drying the cake was broken up and sieved to a 10-20 mesh. These particles were placed in the oxidizer tube of the circuit of the fuel-air ratio indicator, with a layer of drying agent at either end and were then activated by the passage of a stream of dry air through the oxidizer at 150° C. for four hours.

*Example 2.*—A product consisting of the mixed oxides of silver and manganese was prepared as follows: 50 c.c. of water were added to 136 grams of powdered potassium permanganate. 600 c.c. of concentrated nitric acid were then slowly added but with vigorous stirring, the temperature of the reaction being kept below 60° C. The mixture was poured into a large bottle and washed by decantation until there was no further test for nitrates. Then it was washed several times with distilled water and filtered by suction, then dried in an oven at 125° C. for ten to twelve hours. The resulting black powder was added to a solution of 37 grams of silver nitrate in 2 litres of distilled water, and silver oxide was precipitated with sodium or potassium hydroxide, the resulting material after settling being washed and filtered and further treated as in Example 1.

*Example 3.*—A product consisting of the oxides of silver, cobalt and nickel was prepared as follows: 63 grams of nickelous nitrate and 65 grams cobaltous nitrate were dissolved in two gallons of water and the solution was saturated with chlorine. Concentrated sodium hydroxide was added to the solution while continuously bubbling chlorine therethrough precipitating cobaltic and nickelic oxides. After settling, the material was washed by decantation until there was no test for chloride or nitrate. It was then washed several times with distilled water and filtered by suction, then dried in an oven at 200° C. for twelve hours. The dried material was pulverized and added to a solution of 37 grams of silver nitrate in 2 litres of distilled water. Silver oxide was then precipitated with sodium or potassium hydroxide and proceeded with as in Example 1.

These substances were used in the oxidizer tube of the circuit shown in Fig. 1, in which the exhaust from the engine is shown at 1. The sampling conduit 2 extends into this exhaust and leads to a desiccator 3 from which the gas sample is passed through conduit 4 to the oxidizer tube 5, then through conduit 6 into the analyzer 7, and from there through conduit 8 into the gas bubbler 9 from which it is discharged into the air through gas outlet 10. The analyzer 7 may be of any form such as shown for example in detail in the patent above referred to. The electrical connections 11 for supplying the direct current potential to the analyzer and the connec-

tions 12 from the indicator 13 are passed through a cable 14 to the analyzer.

The details of the oxidizer tube may be seen in Figures 2 and 3. The body 15 of the oxidizer is cylindrical in shape and has 3 radial walls 16 as shown forming passages AB, BC, and AC. This construction permits a three-pass gas flow in the length of one pass and each pass utilizing the thermal conditions of the other passages to assist the completion of the reaction. Radial walls A and B are welded to the end plate at the gas entrance 17 whereas radial wall C is shortened here to allow passage of the gas from passage BC to passage AC. Radial walls A and C are welded to the end plate at the gas exit 18 whereas radial wall B is shortened to allow passage of the gas from passage AB to passage BC. The sample gases enter this oxidizer through inlet 19 and leave it by way of outlet 18. At the inlet and outlet is placed some desiccant material so as to keep the oxidant which completely fills the rest of the oxidizer passages free from moisture. At the inlet and outlet is placed some desiccant material so as to keep the oxidant which fills the rest of the body of the oxidizer passage free from moisture.

Thus it may be seen that we have a simple form of analyzer system for determining the fuel-air ratio of the mixture fed to any engine, to the exhaust of which this analyzer is applied. This analyzer is easy to service because the oxidant used is of the type which operates at normal temperatures. It does not require any heating means such as previously used and therefore the oxidizer tube may be positioned so that it is easily accessible for replacement purposes. The oxidizer tube including the oxidant may be made replaceable so that as one oxidant is used up and becomes ineffective a new oxidizer tube with fresh oxidant all ready for operation may be readily substituted.

Obviously various modifications may be made in arrangement of the parts of our circuit, and different forms of the elements may be used without departing from the spirit of the invention, the scope of which is defined by the appended claim.

This invention may be used by or for the Government of the United States of America for governmental purposes without the payment of any royalties thereon or therefor.

What we claim is:

A combined gas oxidizing and desiccating unit comprising a hollow cylindrical body closed at both ends, a gas inlet port in one end, an outlet port in the other end, three longitudinally extending walls within said hollow cylindrical body in equi-angular spaced relationship to each other and radiating from the longitudinal axis to the sidewalls of said cylindrical body, the first of said walls in sealed relationship to both ends of said cylindrical body, the second of said walls in sealed relationship to said one end and terminated short of said other end thereby forming a port between said second wall and said other end, the third of said walls in sealed relationship to said other end and terminated short of said one end thereby forming a port between said third wall and said one end, the said inlet port communicating with the passageway formed by the said first and second walls and said cylindrical body and the said outlet port communicating with the passageway formed by said first and third walls and said cylindrical body whereby a continuous three passageway is formed between said inlet

and outlet ports, said three pass passageway adapted to be substantially filled with an oxidizing agent.

HAROLD C. GERRISH.

JAMES LAWRENCE MEEM, JR.

**REFERENCES CITED**

The following references are of record in the file of this patent:

**UNITED STATES PATENTS**

| Number    | Name | Date          |
|-----------|------|---------------|
| 1,578,666 | Katz | Mar. 30, 1926 |

| Number       | Name             | Date          |
|--------------|------------------|---------------|
| 1,675,228    | Schmidt          | June 26, 1928 |
| 1,744,415    | Pick             | Jan. 21, 1930 |
| 1,992,747    | Gilliland et al. | Feb. 26, 1935 |
| 2,002,525    | Cambron et al.   | May 28, 1935  |
| 2,005,036    | Howe             | June 18, 1935 |
| 2,042,646    | Willenborg       | June 2, 1936  |
| 2,204,431    | Moore et al.     | June 11, 1940 |
| 2,245,531    | Payne            | June 10, 1941 |
| 10 2,298,288 | Gerrish et al.   | Oct. 13, 1942 |
| 2,315,525    | Hulsberg         | Apr. 6, 1943  |
| 2,345,219    | Sanderson        | Mar. 28, 1944 |